# EUROPEAN PATENT SPECIFICATION

(11) **EP 2 279 324 B1**
(45) Date of publication and mention of the grant of the patent: **21.05.2014**
(21) Application number: 09722007.3
(22) Date of filing: 20.03.2009
(51) Int. Cl.: E21B 4/02, E21B 17/00, E21B 17/18, F04C 2/107, F04C 15/00, F04C 13/00

(54) **STATOR FOR USE IN HELICOIDAL MOTOR**
STATOR ZUR VERWENDUNG IN EINEM SCHRAUBENMOTOR
STATOR POUR MOTEUR HÉLICOÏDAL

(30) Priority: 20.03.2008 GB 0805250
(43) Date of publication of application: 02.02.2011
(73) Proprietor: Advanced Interactive Materials Science Limited, Edgbaston Birmingham B15 3BH (GB)
(72) Inventor: ARCHER, Geoffrey, Frederick, Lincolnshire PE9 4BA (GB)
(74) Representative: Barnes, Colin Lloyd
(86) International application number: PCT/GB2009/000754
(87) International publication number: WO 2009/115819

(56) References cited:
- EP-A1- 1 657 010
- EP-A2- 0 815 995
- WO-A1-94/11140
- WO-A1-99/58273
- WO-A2-01/44615
- WO-A2-97/40777
- FR-A1- 2 796 322
- JP-A- 63 312 902
- US-A- 3 975 121
- US-A- 3 992 202
- US-A- 5 171 139
- US-A- 5 832 604
- US-A1- 2005 214 156
- US-A1- 2008 025 859
- BOCANEGRA-BERNAL M H: "Hot Isostatic Pressing (HIP) technology and its applications to metals and ceramics", JOURNAL OF MATERIALS SCIENCE, SPRINGER NETHERLANDS, NL, vol. 39, 1 November 2004 (2004-11-01), pages 6399-6420, XP002532837, ISSN: 0022-2461, DOI: DOI:10.1023/B:JMSC.0000044878.11441.90

## Description

This invention relates to stators for use in helicoidal motors used in down-hole drilling.

Down-hole drilling heads are often driven by a helicoidal motor positioned close to the drilling head and operated by a mud pump. The helicoidal motor comprises a stator coupled to the drill string, and a rotor coupled to the drilling head.

Such helicoidal motors work under very arduous conditions. US 2008 025859 discloses resilient material stators.

We have appreciated that in various circumstances there would be advantage in providing a hole in the stator, for example to accommodate a communications link and/or fluid flow.

It has not previously been possible to create a hole through a metal stator manufactured from the advanced materials that are required to provide a metal stator suitable to resist the abrasive, corrosive and erosive conditions to which a down-hole drilling stator is subjected in use, since such metals cannot be drilled except for creating very short holes.

According to one aspect we provide a stator for a helicoidal down-hole drilling motor, the stator being formed with a through-hole, in addition to the main stator bore.

The stator is preferably produced by a powder metallurgy process.

The hole may extend in any direction through the stator. In particular the hole may be a straight hole extending parallel to the axis of the stator, or the hole may be of helical form, the helix extending about the axis of the stator.

The invention thus provides a hole through the stator part of the linear motor/pump through which information can be transmitted either way to control and/or collect data and information.

The information can be transmitted via electrically conductive materials and/or optical fibres. More than one hole can be placed through the metal stator at a size that does not undermine the strength of the stator but optimises the potential uses of such a hole.

Potentially, but not essentially, the hole can be used for other things including cooling, and/or fluid transmission in addition to transmission of signals in electrical and optical form. In such an instance the hole may, but not essentially, follow the helical form of the internal shape of a stator provided internally with one or more helical flutes.

Such information transmitted through the hole can be typically but not essentially restricted to the collection of temperature, pressure, flow rate, load torque and vibration. It can also be seen that such a hole could provide the means of controlling aspects of a drilling head in such a way that is currently not available in association with a metal stator.

According to an aspect of the invention according to claim 1 a method of producing a net or near net-shape helicoidal motor stator from metal-based powder comprises producing an insert of accurate dimensions corresponding to the dimensions of a main stator bore to be created in the finished stator, the bore having a length of at least 750mm, supporting the insert within a mould cavity, filling the mould cavity with metal-based powder, subjecting the powder to isostatic pressing, and subsequently removing the material of the insert.

As is well known, the mould may be an independent mould that is removed after an initial step to bind the powder together into a pre-form, and the pre-form is then encapsulated in a suitable containment which may be a canister or a sprayed coating, or a canister of suitable internal shape may be used as the mould, and the canister itself is evacuated prior to HIPing

Preferably the insert is supported in position in the mould cavity by a plurality of formers of a material that is compatible with the finally consolidated powder.

The insert may be a metallic insert of a material that is subsequently removable by chemical etching, preferably copper. The chemical etching may be assisted by electrolytic reaction.

In suitable cases the insert need only be coated with a material that can subsequently be removed by etching, in order to release the insert, which can then be extracted.

Preferably the metallic insert is coated with a suitable material that provides a diffusion barrier to prevent the material of the insert from diffusing by atomic diffusion into the powder being consolidated during HIPing.

The invention can enable a helical bore to be provided in a stator.

In one preferred embodiment a copper rod, of a diameter in the range of 6 to 10 mm for example and of length greater than 2m, is first bent into a helix of the required dimensions and this is then held in position in a powder containment prior to filling the containment with powder. The containment enclosing the powder, rod and former, is then consolidated by solid state diffusion using the HIPing method.

The diffusion barrier may be Al₂O₃ applied by vapour phase deposition or by high velocity spraying. Alternatively, the diffusion barrier may be created by applying boron nitride as an aqueous solution by spraying.

In a second embodiment a preformed metal tube, of 6mm to 10mm diameter for example, is filled with ceramic particles and is bent to a helical shape and placed within the powder containment prior to filling the containment with powder. The tube is held in position with formers compatible with the finally consolidated powder. The entire containment encompassing the metallic and/or cermet/MMC powder is then consolidated by solid state diffusion using the HIPing method.

During consolidation the metal tube may become totally diffusion bonded into the consolidated component but the ceramic particles will remain in the pre-process particle form and thereby can be removed mechanically via vibration techniques to leave a clean hole through the component.

### Example

The invention can be used to provide one or more holes in one or more helical lobes provided internally of a stator body having a length of as much as 2m or more. The hole or holes can be positioned to follow the core of a helical flute, which may have a pitch of about 1m and a radius of 50mm about the body axis. The helical lobes are defined by helical grooves in a mandrel that is positioned in the mould during pressing of the stator body.

## Claims

1. A method of producing a net or near net-shape helicoidal motor stator from metal-based powder, the stator having a main stator bore and a through-hole in addition to the main stator bore, the method comprising producing an insert of accurate dimensions corresponding to the dimensions of the main stator bore to be created in the finished stator, the bore having a length of at least 750mm, supporting the insert within a mould cavity, filling the mould cavity with metal-based powder, subjecting the powder to isostatic pressing, and subsequently removing the material of the insert.

2. The method of claim 1 in which the mould is an independent mould that is removed after an initial step to bind the powder together into a pre-form, and the preform is then encapsulated in a suitable containment.

3. The method of any one of claims 1 or 2 in which the insert is a metallic insert of a material that is subsequently removable by chemical etching.

4. The method of claim 3 in which the insert comprises copper.

5. The method of any one of the claims 3 or 4 in which the metallic insert is coated with a material that provides a diffusion barrier to prevent the material of the insert from diffusing by atomic diffusion into the powder being consolidated during HIPing.

6. The method of claim 5 in which the diffusion barrier comprises Al₂O₃ applied by vapour phase deposition or high velocity spraying.

7. The method of claim 5 in which the diffusion barrier is created by applying boron nitride as an aqueous solution by spraying.

8. The method of claim 1 in which the insert is produced by taking a preformed metal tube, of 6mm to 10mm diameter, filling the tube with ceramic particles, and bending the filled tube to a helical shape, placing the helical filled tube within the powder containment prior to filling the containment with powder, holding the tube in position with formers compatible with the finally consolidated powder, providing a containment encompassing the metallic and/or cermet/MMC powder, consolidating the contained material by solid state diffusion using a HIPing method and then removing the ceramic particles mechanically by a vibration technique to leave a clean hole through the finished component.

## Patentansprüche

1. Verfahren zum Herstellen eines netzförmigen oder nahezu netzförmigen schraubenartigen Motorstators aus einem Pulver auf Metallbasis, wobei der Stator eine Hauptstatorbohrung und eine durchgehende Bohrung zusätzlich zur Hauptstatorbohrung aufweist, wobei das Verfahren umfasst: Erzeugen einer Einlage mit exakten Abmessungen, die den Abmessungen der Hauptstatorbohrung entsprechen, die im fertigen Stator ausgebildet werden soll, wobei die Bohrung eine Länge von mindestens 750 mm aufweist, Stützen der Einlage in einer Formkavität, Füllen der Formkavität mit dem Pulver auf Metallbasis, isostatisches Pressen des Pulvers und anschließend Entfernen des Materials der Einlage.

2. Verfahren nach Anspruch 1, bei dem die Form eine unabhängige Form ist, die nach einem Anfangsschritt, in dem das Pulver zu einem Vorformling verbunden wird, entfernt wird, und der Vorformling dann in einer geeigneten Hülle eingekapselt wird.

3. Verfahren nach einem der Ansprüche 1 oder 2, wobei die Einlage eine metallische Einlage aus einem Material ist, das anschließend durch chemisches Ätzen entfernt werden kann.

4. Verfahren nach Anspruch 3, wobei die Einlage Kupfer umfasst.

5. Verfahren nach einem der Ansprüche 3 oder 4, wobei die metallische Einlage mit einem Material beschichtet ist, das eine Diffusionsbarriere bereitstellt, um zu verhindern, dass das Material der Einlage durch atomare Diffusion in das Pulver diffundiert, das sich während einer HIP-Behandlung verfestigt.

6. Verfahren nach Anspruch 5, bei dem die Diffusionsbarriere Al₂O₃ umfasst, das durch Dampfphasenabscheidung oder Hochgeschwindigkeitssprühen aufgebracht wird.

7. Verfahren nach Anspruch 5, bei dem die Diffusionsbarriere durch Aufbringen von Bornitrid als wässrige Lösung durch Sprühen aufgebracht wird.

8. Verfahren nach Anspruch 1, bei dem die Einlage durch Nehmen eines vorgeformten Metallrohrs mit einem Durchmesser von 6 mm bis 10 mm, Füllen des Rohrs mit keramischen Teilchen und Biegen des gefüllten Rohrs in eine Schraubenform, Einbringen des schraubenförmigen gefüllten Rohrs in die Pulverhülle vor dem Befüllen der Hülle mit Pulver, Festhalten des Rohrs mit Formeinrichtungen, die mit dem endgültig verfestigten Pulver kompatibel sind, Bereitstellen einer Hülle, die das metallische und/oder Cermet/MMC-Pulver einschließt, Verfestigen des umhüllten Materials durch Festzustandsdiffusion unter Verwendung eines HIP-Verfahrens und anschließend mechanisches Entfernen der keramischen Partikel durch eine Rütteltechnik, um ein sauberes durchgehendes Loch in der fertigen Komponente zu hinterlassen.

## Revendications

1. Un procédé de production d'un stator de moteur hélicoïdal en forme de filet ou quasi filet à partir d'une poudre métallique, le stator possédant un trou traversant en plus de l'orifice de stator principal, le procédé comprenant la production d'un insert de dimensions exactes correspondant aux dimensions de l'orifice de stator principal à créer dans le stator terminé, l'orifice possédant une longueur d'au moins 750 mm, l'appui de l'insert à l'intérieur d'une cavité de moule, le remplissage de la cavité de moule avec une poudre métallique, la soumission de la poudre à une compression isostatique, et ensuite l'élimination du matériau de l'insert.

2. Le procédé selon la Revendication 1 dans lequel le moule est un moule indépendant qui est retiré après une opération initiale de liaison de la poudre en une préforme, et la préforme est ensuite encapsulée dans une enceinte adaptée.

3. Le procédé selon l'une quelconque des Revendications 1 ou 2 dans lequel l'insert est un insert métallique d'un matériau qui peut ensuite être éliminé par gravure chimique.

4. Le procédé selon la Revendication 3 dans lequel l'insert contient du cuivre.

5. Le procédé selon l'une quelconque des Revendications 3 ou 4 dans lequel l'insert métallique est enduit avec un matériau qui fournit une barrière de diffusion destinée à empêcher le matériau de l'insert de se diffuser par diffusion atomique dans la poudre qui est consolidée au cours du procédé de compression isostatique à chaud (HIP).

6. Le procédé selon la Revendication 5 dans lequel la barrière de diffusion contient du Al₂O₃ appliqué par dépôt en phase vapeur ou pulvérisation haute vitesse.

7. Le procédé selon la Revendication 5 dans lequel la barrière de diffusion est créée par l'application de nitrure de bore sous la forme d'une solution aqueuse par pulvérisation.

8. Le procédé selon la Revendication 1 dans lequel l'insert est produit par la prise d'un tube métallique préformé de 6 à 10 mm de diamètre, le remplissage du tube avec des particules de céramique et le pliage du tube rempli selon une forme hélicoïdale, le placement du tube rempli hélicoïdal à l'intérieur de l'enceinte à poudre avant le remplissage de l'enceinte avec de la poudre, le maintien du tube en position avec des gabarits compatibles avec la poudre consolidée finale, la fourniture d'une enceinte englobant la poudre métallique et/ou le cermet/MMC, la consolidation du matériau contenu par diffusion à l'état solide au moyen d'un procédé de compression isostatique à chaud (HIP) et ensuite l'élimination des particules de céramique mécaniquement par une technique de vibration de façon à laisser un trou propre au travers du composant terminé.
